

## UNITED STATES PATENT OFFICE

LODEWIJK PIETER FRANS VAN DER GRINTEN AND KAREL JAN JOSEPH VAN DER GRINTEN, OF VENLO, NETHERLANDS, ASSIGNEES TO N. V. CHEMISCHE FABRIEK L. VAN DER GRINTEN, OF VENLO, NETHERLANDS, A DUTCH COMPANY

## MANUFACTURE OF SENSITIVE DIAZO-TYPE LAYERS

No Drawing. Application filed May 12, 1930, Serial No. 451,837, and in the Netherlands May 15, 1929.

It is known to make direct positive prints from positives by means of the diazo type process. It is also known that the development and fixing of the prints can take place in one action by simple addition of a substance (or substances).

This addition of substances can be effected by treating the prints with a gas or a liquid. The treatment with gas is limited to the addition of alkali only, and the sensitive layer must consequently contain the azo-component. In the case of treatment with liquid, this limitation does not exist, and the paper may contain only the diazo compound (in which case the developer contains alkali plus azo-component) or it may contain both components (in which case the developer contains alkali but no azo-component). Each method (gas or liquid) has its advantages and disadvantages.

Of late, the liquid development has gained ground in practice, this method having been improved by U. S. Patents No. 1,841,653 and No. 1,821,306 and U. S. patent application Serial No. 353,248. The treatment is rapid, simple and inodorous, and makes it possible to apply reducing agents which prevent yellowing, but are not stable against acid, and also to apply a sizing agent with the developer.

In the practice of the liquid method (since the introduction of the process according to U. S. Patent No. 1,841,653, also called the "half wet" method) the following difficulty is encountered:

It is desirable that the developer shall have a simple composition. This might be obtained by incorporating the azo-component in the sensitive layer so that it can be omitted from the developer. According to the known processes in which this is effected, viz. that of U. S. Patent No. 1,444,469 or German Patent No. 422,972 or British Patent No. 234,818, the mixture of diazo compound and azo-component, forming the sensitive layer, must be a slowly reacting mixture, as otherwise coupling during storage before use cannot be prevented. According to the known processes coupling is prevented chiefly by using slow-coupling (slightly active) diazo compounds,

such as "diazo-anhydrides" (vide U. S. Patent No. 1,444,469), "diazo-anhydrides in a broader sense" (vide German Patent No. 422,972), "diazo compounds which will not couple per se in an acid or neutral condition with any azo-dyestuff component" (vide British Patent No. 234,818). If it is desired to develop prints on such layers by applying a thin uniform layer of a liquid developer (U. S. Patent No. 1,841,653), for example with an apparatus as described in U. S. Patent No. 1,821,306, the difficulty is encountered that owing to the slowness of the coupling reaction the separate substances of the layer dissolve in the liquid and spread more or less before the coupling is finished. The coupling is therefore complete only after this spreading has taken place, so that pigments are formed in the parts that have spread.

In this manner the pictures obtained are blurred, and in some cases have streaks in the background. This difficulty is reduced to a minimum by the process according to U. S. Patent No. 1,841,653 and with the apparatus according to U. S. Patent No. 1,821,306, but only sufficiently for quick-coupling combinations, and not for the slow-coupling combinations of U. S. Patent No. 1,444,469, German Patent No. 422,972 and British Patent No. 234,818.

These combinations can be developed with a very concentrated alkaline liquid, which promotes quick coupling by reason of its concentration, but in this case the support of the picture, the fibres and sizing of the paper are damaged, and the finished picture is liable to become very yellow. With these combinations the spreading of the colours can also be prevented to some extent by other more or less complicated and detrimental means, for example by using developers which contain large quantities of salts, or developers in alcoholic solution. However, all these processes have considerable practical disadvantages.

As already stated, with quick-coupling combinations it is necessary, on account of the stability, to apply both components separately, the diazo-component being in the sensitive layer, and the azo-component being in the developer, so that these combinations are es-

55

60

65

70

75

80

85

90

95

100

sentially distinguished from those of the above mentioned patent specifications.

- It has been found that with the quick-coupling combinations necessary for the "half wet" development as above described, light-sensitive layers containing both components may be used, provided the layers are completely or approximately completely dried. Here it may be observed that normal dry paper has a moisture content of 5% or more. Light-sensitive papers, including blue print paper, but more especially diazo-type papers for ammonia development, have a moisture content of about 6%. With diazo-type paper for gaseous development this moisture content is even a "conditio sine qua non", as the paper would not couple or would couple only very incompletely in gaseous ammonia if in a perfectly dry condition.
- The moisture content, with which the above mentioned quick-coupling combinations may be used in light-sensitive layers containing both components, while maintaining a practically sufficient stability against coupling, is under 3-4%. In practice, a moisture content of 1-2% can be reached, and a paper of very good stability is thus obtained.

As stated above, the combinations according to U. S. Patent No. 1,444,469, German Patent No. 422,972, British Patent No. 234,818 and the patents corresponding therewith, are made too slow-coupling for gaseous development when they are prepared with a moisture content under 6%. Restoration of a sufficient moisture content in order to obtain adequate development cannot take place, or only insufficiently or in a very cumbrous manner. If a paper according to U. S. Patent No. 1,444,469, German Patent No. 422,972, British Patent No. 234,818 and the patents corresponding therewith has been wholly dried, the restoration of the coupling velocity (development velocity) sufficient for gaseous development, necessitates a prolonged stay in a moist atmosphere, unless the moisture content is increased, for example by steam or the like, which is however too cumbrous for practical purposes.

The same difficulties are met when an attempt is made to develop the above described strongly dried quick-coupling combinations with gases (although in a considerably smaller degree, because the combination couples more quickly). With the liquid development, however, no difficulty is encountered, for in this case not only the chemical agent (alkali) which effects the coupling, but also the water necessary for the reaction, is supplied by the developer. Consequently, two factors are combined, which form the essential feature of the present invention.

On the one hand layers having both components in an active coupling combination are used, whilst the activity necessary for the

later development is temporarily (during storage) taken away from this combination by maintaining a very low moisture content.

On the other hand, even by the liquid development the substance (water) is automatically supplied, which failed for the possibility of coupling. Consequently, in the development of these layers not only the alkali is active, but also the water, which is indispensable for the reaction. These layers can be developed therefore practically only by water plus alkali, or in other words, only with an aqueous solution of alkali.

The stability of these layers, which consequently contain both substances of an actively coupling combination of diazo- and azo-components is, as explained above, due to the low moisture content. A characteristic feature of these layers is that even after one or several days, they show a detrimental deterioration (by premature coupling) if the moisture content rises to or exceeds the normal (6%), for example if they are kept in a bad or defective packing in a moist warm summer atmosphere. Consequently care must be taken to provide a final moisture-proof packing, which however is easily realized in practice.

In order to increase the stability of the layers, known means for counteracting the coupling may be used, such as acids, mixtures of acids or acid reacting substances in the mass of the support. Also substances may be used which are capable of combining with water in the form of water of crystallization, such as wholly or partly dehydrated aluminium sulphate or alum or other salts, also substances acting on the azo-component, such as hydroxylamine, semicarbazide and the like. However, these latter means have more or less the result of only displacing the difficulty, as they hinder or delay the coupling in a manner which cannot be rectified by the developer with the same velocity as the absence of moisture. The reducing substances for preventing the yellowing of the diazo-types, described in U. S. Patent No. 1,821,281 may also be added to the light-sensitive layers according to the invention. The addition of salts to the sensitive layers may further increase the sharpness of the pictures. The presence of salts which act as buffers to an alkali, such as ammonium salts, either in the sensitive layer or in the body of the support, diminishes the detrimental effect of the alkaline developer on the sizing and the yellowing. Salts forming sparingly soluble compounds with the diazo compound, such as sodium chlorostannate, cadmium and zinc salts, increase the sharpness of the picture, as they better localize the diazo compound. Moreover, they have also a somewhat beneficial effect on the durability, as they influence favourably the localization and separation of the components, obtained by drying,

- which tends to prevent coupling. Of course, insoluble diazo compounds have the same advantage, but these are technically more difficult to bring into a light-sensitive layer.
- 5 Good localization of the substances of the layer is assisted by having the solutions of the ingredients thoroughly absorbed in the support, for example paper, before subjecting to the intense drying. Owing to the intense drying according to this invention, the paper (if prepared in this manner) becomes naturally brittle. This brittleness, however, is wholly or mainly removed by the "half wet" treatment on development. After this treatment the paper nearly regains its original tenacity.

*Example 1*

Paper containing an excess of alum is pre-  
20 treated with a solution of 3% sodium chloro-  
stannate, thereafter covered with a solution  
containing: 1% 1-dibenzylamido benzene-4-  
diazonium chloride (prepared by diazotizing  
para dibenzylamido-aniline), 2% thiocar-  
bamide, 1.2% hydroxylamine sulphate, 5%  
25 glucose, 2% oxalic acid, 1% gelatine, 5% am-  
monium chloride, 0.2% phloroglucinol and  
0.2% resorcinol.

After a short absorption the paper is in-  
30 tensively dried until the moisture content  
has fallen to about 2% (defined by loss of  
weight on completely drying at high tem-  
perature). This paper is sufficiently stable  
for practical purposes, provided it remains  
35 completely dry. After exposure under a  
transparent original, the paper is developed  
in an apparatus according to U. S. Patent  
No. 1,821,306 with a solution of 3½% sodi-  
um carbonate, 5% sodium thiosulphate and  
40 5% sodium citrate.

A strong positive image on a white ground  
is obtained which ground does not become  
yellow. It is also possible to use ordinary  
45 paper and to omit the pretreatment. The  
paper is then somewhat less stable and the  
prints become a little more yellow. Also the  
thiocarbamide and glucose may be left out  
of the layer, and the thiosulphate and citrate  
may be left out of the developer, resulting  
50 however, in yellowing. If the hydroxyl-  
amine and oxalic acid are omitted the paper  
becomes somewhat less stable, but in that case  
a weaker alkali can be used for developing,  
and after development the sizing is better.  
55 If ammonium chloride or gelatine is omit-  
ted, the sizing becomes somewhat worse after  
development.

*Example 2*

60 Paper is brushed on the back with a 10%  
solution of ammonium chloride, and then on  
the front with a solution containing: 1% 1-  
di-isoamylamine benzene-4-diazonium chlo-  
rostannate (prepared by diazotizing para-  
65 di-isoamylaniline and adding tin chloride

and strong hydrochloric acid), 2% thiocar-  
bamide, 2% phosphoric acid, 1% gelatine,  
0.2% phloroglucinol, 0.2% resorcinol.

The paper is intensively dried until the  
moisture content has fallen to about 2%.  
70 The paper has a sufficient stability, provided  
absorption of moisture is prevented. After  
exposure the development takes place as de-  
scribed in Example 1. The omission of vari-  
ous substances has the same effect as in Ex-  
75 ample 1. A strong positive picture is ob-  
tained.

*Example 3*

Paper is covered with a solution of: 2%  
3 - diazo - hexahydrocarbazol-chlorostannate  
80 (prepared by diazotizing 3 - amino - hexa-  
hydrocarbazol and adding tin chloride in  
strong hydrochloric acid), 2% thiocarba-  
mide, 2% hydroxylamine sulphate, 1% semi-  
carbazide chloride, 2% tartaric acid, 5%  
85 sodium citrate, 5% sodium chloride, 0.2%  
phloroglucinol.

The paper is intensively dried until the  
moisture content has fallen below 2%. The  
90 paper is of a scarcely sufficient stability.  
After exposure the paper is developed as de-  
scribed in Example 1 with a solution of 2%  
soda, 10% sodium thiosulphate.

The development can also take place with  
a bicarbonate solution, sodium borate and  
the like. A strong positive picture is ob-  
95 tained. Certain substances may be omitted  
as described in Example 1.

If the citrate and sodium chloride are  
100 omitted from the layer, somewhat less sharp  
pictures are obtained.

What we claim is:—

1. The process for preparing a base hav-  
ing a light sensitive diazo type layer there-  
105 on which comprises applying a rapidly cou-  
pling mixture of a diazo compound and an  
azo dyestuff component to said base, and  
drying the base until the moisture content  
thereof is reduced to a point not exceeding  
110 4% of its dry weight.

2. The process according to claim 1 where-  
in the diazo compound is a diazochlorostan-  
nate.

3. The process for preparing a base hav-  
ing a light sensitive diazo type layer there-  
115 on which comprises applying a buffering  
agent and a rapidly coupling mixture of a  
diazo compound and an azo dyestuff compo-  
nent to said base, and drying the base until  
the moisture content thereof is reduced to a  
120 point not exceeding 4% of its dry weight.

4. The process according to claim 3 where-  
in the buffering agent is an ammonium salt.

5. The process according to claim 3 where-  
125 in the diazo compound is a diazochlorostan-  
nate.

6. The process for preparing a base having  
a light sensitive diazo type layer thereon  
which comprises applying a rapidly coupling  
130

- mixture comprising a diazo compound, an azo dyestuff component, and a substance capable of arresting the coupling activity of said mixture to said base, and drying the base 5 until the moisture content thereof is reduced to a point not exceeding 4% of its dry weight.
7. The process according to claim 6 wherein the substance is an acidic substance.
8. The process according to claim 6 where- 10 in the substance is a salt capable of combining with water in the form of water of crystallization.
9. The process according to claim 6 where- 15 in the substance is hydroxylamine.
10. The process according to claim 6 wherein the diazo compound is a diazochlorostan- nate.
11. The process for preparing a base hav- 20 ing a light sensitive diazo type layer thereon which comprises applying a rapidly coupling mixture comprising a diazo compound, an azo dyestuff component, and a reducing agent capable of arresting the discoloration of the background of the finished print, and drying 25 the base until the moisture content thereof is reduced to a point not exceeding 4% of its dry weight.
12. The process according to claim 11 wherein the diazo compound is a diazochloro- 30 stannate.
13. The process for preparing a base hav- 35 ing a light sensitive diazo type layer thereon which comprises applying a rapidly coupling mixture comprising a diazo compound, an azo dyestuff component, and a salt capable of forming with said diazo compound a difficultly soluble salt, and drying the base until the moisture content thereof is reduced to a point not exceeding 4% of its dry weight.
14. The process according to claim 13 wherein the diazo compound is a diazochloro- 40 stannate.
15. As a new product, a base having there- 45 on a sensitive layer comprising a rapidly coupling mixture of a diazo compound and an azo dyestuff component, said base having the moisture content reduced to a point not exceeding 4% of its dry weight.
16. As a new product, a base having there- 50 on a sensitive layer comprising a rapidly coupling mixture of a diazo compound and an azo dyestuff component, said base having its moisture content reduced to less than 3% of its dry weight.
17. As a new product, a base having a sen- 55 sitive layer comprising a buffering agent and a rapidly coupling mixture of a diazo compound and an azo dyestuff component thereon, said base having the moisture content 60 reduced to a point not exceeding 4% of its dry weight.
18. As a new product, a base having a sen- 65 sitive layer comprising a rapidly coupling mixture of a diazo compound and an azo dy- stuff component and a substance capable of arresting the coupling activity of said mixture, said base having the moisture content reduced to a point not exceeding 4% of its dry weight.
19. The product according to claim 18 70 wherein the substance is an acidic substance.
20. The product according to claim 18 wherein the substance is hydroxylamine.
21. As a new product, a base having there- 75 on a sensitive layer comprising a rapidly coupling mixture of a diazo compound and an azo dyestuff component and a salt capable of forming with said diazo compound a difficultly soluble salt, said base having the moisture content reduced to a point not exceeding 80 4% of its dry weight.
22. The product according to claim 21 wherein the diazo compound is a diazochloro- stannate.
23. A process for preparing a base having 85 a light sensitive diazotype layer thereon, which comprises impregnating the base with a buffering agent and applying a rapidly coupling mixture of a diazo compound and an azo dyestuff component to the surface of said base, and drying the base until the moisture content thereof is reduced to a point not exceeding 4% of its dry weight.
24. A process for preparing a base having 90 a light sensitive diazotype layer thereon, which comprises impregnating the base with an acidic substance and applying a rapidly coupling mixture of a diazo compound and an azo dyestuff component to the surface of said base, and drying the base until the moisture content thereof is reduced to a point not exceeding 4% of its dry weight.
25. A process for preparing a base having 95 a light sensitive diazotype layer thereon, which comprises impregnating the base with a salt capable of arresting bleeding of the print upon contact with the development liquid, and applying a rapidly coupling mixture of a diazo compound and an azo dy- 100 estuff component to the surface of said base, and drying the base until the moisture content thereof is reduced to a point not exceeding 4% of its dry weight.
26. A process for preparing a base having 105 a light sensitive diazotype layer thereon, which comprises impregnating the base with a salt capable of forming upon reaction with a diazo compound a difficultly soluble com- 110 pound, and applying a rapidly coupling mixture of a diazo compound and an azo dy- 120 estuff component to the surface of said base, and drying the base until the moisture content thereof is reduced to a point not exceeding 4% of its dry weight.
- In testimony whereof we affix our signa- 125 tures.
- LODEWIJK PIETER FRANS van der GRINTEN.  
KAREL JAN JOSEPH van der GRINTEN.